# EUROPEAN PATENT SPECIFICATION

(11) **EP 2 184 371 B1**
(45) Date of publication and mention of the grant of the patent: **30.11.2016**
(21) Application number: 08791572.4
(22) Date of filing: 24.07.2008
(51) Int. Cl.: C22C 9/06, C22C 9/02, C22C 9/00, C22F 1/08, H01R 13/03, H01R 13/11, H01R 43/16

(54) **COPPER ALLOY SHEET**
KUPFERLEGIERUNGSBLECH
FEUILLE D'ALLIAGE DE CUIVRE

(30) Priority: 07.08.2007 JP 2007205630; 07.09.2007 JP 2007232641; 27.09.2007 JP 2007252036; 27.09.2007 JP 2007252037
(43) Date of publication of application: 12.05.2010
(62) Divisional of application: 13005147.7
(73) Proprietor: Kabushiki Kaisha Kobe Seiko Sho, Chuo-ku, Kobe-shi, Hyogo 651-8585 (JP)
(72) Inventor: ARUGA, Yasuhiro, Kobe-shi, Hyogo 651-2271 (JP); HASHIMOTO, Daisuke, Shimonoseki-shi, Yamaguchi 752-0953 (JP); NOMURA, Koya, Shimonoseki-shi, Yamaguchi 752-0953 (JP)
(74) Representative: Müller-Boré & Partner Patentanwälte PartG mbB
(86) International application number: PCT/JP2008/063320
(87) International publication number: WO 2009/019990

(56) References cited:
- EP-A1- 0 859 065
- EP-A1- 1 801 249
- WO-A1-2006/132317
- JP-A- 11 222 641
- JP-A- 62 099 430
- JP-A- 62 099 430
- JP-A- 62 227 052
- JP-A- 62 227 052
- JP-A- 2000 129 377
- JP-A- 2000 256 814
- JP-A- 2001 262 255
- JP-A- 2001 262 297
- JP-A- 2002 180 165
- JP-A- 2002 294 368
- JP-A- 2006 083 465
- JP-A- 2006 342 389
- JP-A- 2007 169 741
- JP-A- 2008 024 994
- US-A- 4 666 667
- US-A- 5 387 293
- US-A1- 2002 108 685

## Description

The present invention relates to a copper alloy sheet. More specifically, the present invention relates to a copper alloy sheet having properties suitable for a connection component such as automotive terminal or connector.

A connection component such as automotive terminal or connector recently requires a performance enough to ensure reliability in a high-temperature environment such as engine room. One of most important properties for the reliability in a high-temperature environment is a contact-fitting force maintaining characteristic, that is, a stress relaxation resistance characteristic.

Fig. 4 shows a structure of a box-type connector (female terminal 3) representative of a connection component such as automotive terminal or connector. Fig. 4(a) is an elevational view and Fig. 4(b) is a cross-sectional view. In Fig. 4, the female terminal 3 has a pressing strip 5 cantilever-supported in an upper holder part 4 and when a male terminal (tab) 6 is inserted into the holder, the pressing strip 5 is elastically deformed and the male terminal (tab) 6 is fixed by the reaction force. Incidentally, in Fig. 4, 7 is a wire connecting part and 8 is an anchoring tongue strip.

As shown in Fig. 4, in the case where a stationary displacement is given to a spring-shaped component composed of a copper alloy sheet and a male terminal (tab) 6 is fitted at a spring-shaped contact part (pressing strip) 5, if the connector is kept standing in a high-temperature environment such as engine room, the contact-fitting force is lost with the lapse of time. Accordingly, the stress relaxation resistance characteristic is such a resistance characteristic against high temperatures as not allowing great reduction in the contact-fitting force of the spring-shaped component composed of a copper alloy sheet even when the connection component is kept standing in a high-temperature environment.

In the SAEJ (the Society of Automotive Engineers of Japan) Standards JASO-C400, as regards the stress relaxation resistance characteristic, the stress relaxation ratio after holding under the conditions of 150°C x 1,000 hr is specified to be 15% or less. Figs. 3(a) and (b) each shows a tester for the stress relaxation resistance characteristic according to this standard. Using this tester, a test specimen 1 cut out into a strip shape is fixed at one end to a rigid test board 2, warped by lifting another end in a cantilever manner (d: warpage size), kept standing at a predetermined temperature for a predetermined time, and then unloaded at room temperature, and the warpage size after unloading (permanent distortion) is determined as δ. Here, the stress relaxation ratio (RS) is represented by RS = (δ/d) x 100.

However, the stress relaxation ratio of a copper alloy sheet has anisotropy and takes a different value according to the direction in which the longitudinal direction of the test specimen runs with respect to the rolling direction of the copper alloy sheet. In this respect, the connection component such as automotive terminal or connector must have a stress relaxation ratio of 15% or less in the direction used as a spring, that is, in either one direction parallel or orthogonal to the rolling direction of the sheet.

As for the copper alloy excellent in the stress relaxation resistance characteristic, a Cu-Ni-Si-based alloy, a Cu-Ti-based alloy, a Cu-Be-based alloy and the like have been heretofore widely known, but in recent years, a Cu-Ni-Sn-P-based alloy having a relatively small additive element content has been used. This Cu-Ni-Sn-P-based alloy allows for ingot making in a shaft furnace which is a large-scale melting furnace with the opening being widely opened to the atmosphere, and because of its high productivity, a great cost down can be achieved.

Also, various techniques for enhancing the stress relaxation resistance characteristic of the Cu-Ni-Sn-P-based alloy itself have been conventionally proposed. For example, Patent Documents 1 and 2 disclose a technique of uniformly and finely dispersing an Ni-P intermetallic compound in a Cu-Ni-Sn-P-based alloy matrix to enhance the electrical conductivity and at the same time, enhance the stress relaxation resistance characteristic and the like, and Patent Documents 2 and 3 disclose a technique of decreasing the P content of a Cu-Ni-Sn-P-based alloy to obtain a solid solution-type copper alloy reduced in the precipitation of an Ni-P compound. Furthermore, Patent Documents 4 and 5 disclose a technique of specifying the substantial temperature and holding time in finish annealing at the production of a Cu-Ni-Sn-P-based alloy sheet to enhance the electrical conductivity and at the same time, enhance the stress relaxation resistance characteristic and the like.
Patent Document 1: Japanese Patent No. 2,844,120
Patent Document 2: Japanese Patent No. 3,871,064
Patent Document 3: JP-A-11-293367 (the term "JP-A" as used herein means an "unexamined published Japanese patent application")
Patent Document 4: JP-A-2002-294368
Patent Document 5: JP-A-2006-213 999

Further, WO 2006/132317 A1 discloses a Cu-Ni-Sn-P based alloy comprising 0.1 to 3.0 mass% of Ni, 0.01 to 3.0 mass% of Sn, 0.01 to 0.3 mass% of P with the remainder being copper and inevitable impurities.

EP 1 801 249 A1 discloses a Cu-Ni-Sn-P based alloy comprising 0.1 to 3.0% of Ni, 0.1 to 3.0% of Sn, and 0.01 to 0.3% of P in mass percent respectively, and the remainder being copper and inevitable impurities, wherein in a radial distribution function around a Ni atom according to a XAFS analysis method, a first peak position is within a range of 2.16 to 2.35 Å, the position indicating a distance between a Ni atom in Cu and an atom nearest to the Ni atom.

JP 2006-342389 A discloses a copper alloy sheet having a composition which is composed of 0.4 to 1.6% of Ni, 0.4 to 1.6% of Sn, 0.027 to 0.15 of P and 0.005 to 0.15% of Fe in mass percent respectively, and the remainder being copper and inevitable impurities, wherein the ratio of the Ni content and P content is < 1.5, wherein the copper alloy sheet has a structure in which precipitates of an Ni-P intermetallic compound are dispersed in the matrix phase of the copper alloy and the precipitates have a diameter of ≤ 60 nm, and ≥ 20 pieces of the precipitates having a diameter of 5 to 60 nm are observed in the region of a visual field of 500 nm x 500 nm.

EP 0 859 065 A1 discloses a copper base alloy for the use in terminals that consists essentially, on a weight basis, of 0.5 to 3.0 % Ni, 0.5 to 2.0 % Sn, 0.010 to 0.20 % P, and optionally 0.01 to 2.0 % Zn, the balance being Cu and incidental impurities.

US-patent 5,387,293 discloses a copper alloy which consists essentially of 1.10 wt. % Ni, 1.48 wt.% Sn and 0.05 wt. % P, with the remainder being Cu and incidental impurities, said alloy having a tensile strength of at least 50 kgf/mm², a spring limit of at least 40 kgf/mm², a stress relaxation of not more than 10% and an electrical conductivity of at least 30% IACS, said copper alloy having uniformly dispersed therein fine particles of a Ni-P compound.

US-patent 4,666,667 discloses a high-strength, high-conductivity phosphor bronze alloy having enhanced resistance to peeling of solder at an elevated temperature consisting essentially of from 0.8 to 4.0% by weight of Sn; from 0.01 to 0.4% by weight of P; from 0.05 to 1.0% by weight of Ni; from 0.05 to 1.0% by weight of Zn; and the remainder of copper and inevitable impurities.

JP 2000-256814 A discloses a copper alloy ingot containing, by weight, 0.2 to 3.0% Ni, 0.5 to 2.0% Sn, 0.01 to 1.0% P, and the balance Cu with inevitable impurities, in which the ratio of Ni (%) to P (%) is smaller than 20.

JP 2001-262255 A discloses a copper based alloy having a composition containing, by weight, 0.2 to 3.0% Ni, ≤2.0% Sn, 0.005 to 2.0% P (or 0.2 to 3.0% Mn, ≤ 2.0% Sn and 0.005 to 2.0% P, or 0.1 to 1.0% Co, ≤ 2.0% Sn and 0.005 to 1.0% P), and the balance Cu with inevitable impurities and having a tensile strength of ≥ 550 MPa, a spring critical value of ≥ 450 MPa, an electric conductivity of ≥ 40% IACS, the minimum bend radius ratio of ≥ 1 and a stress relaxation ratio of ≤ 10%.

JP 2001-262297 A discloses a copper based alloy having a composition containing, by weight, 0.2 to 3.0% Ni, ≤ 2.0% Sn, 0.005 to 2.0% P (or 0.2 to 3.0% Mn, ≤ 2.0% Sn and 0.005 to 2.0% P, or 0.1 to 1.0% Co,≤ 2.0% Sn and 0.005 to 1.0% P), and the balance Cu with inevitable impurities and having a tensile strength of ≤ 550 MPa, a spring critical value of ≥ 450 MPa, an electric conductivity of ≤ 40% IACS, a minimum bending radius ratio of ≤ 1 and a stress relaxation ratio of ≤ 10%.

JP 2000-129377 A discloses a copper based alloy having a composition which consists of, by weight, 0.5 to 3.0% Ni, 0.5 to 2.0% Sn, 0.025 to 1.0% P, and the balance Cu with inevitable impurities and optionally contains 0.01 to 2.0% Zn and in which the ratio between the Ni wt.% and the P wt.% takes a value less than 20 and the alloy has a structure where part of the contained Ni and P are finely and uniformly precipitated in the form of an Ni-P intermetallic compound in a matrix.

However, mechanical properties of these conventional Cu-Ni-Sn-P-based alloys enhanced in the stress relaxation resistance characteristic are such that, for example, when the 0.2%-proof stress is about 500 MPa, the elongation is only less than 10%, and the elongation is low for the strength. Also, as for the terminal/connector properties, while a stress relaxation ratio of 15% or less is achieved in the direction parallel to the rolling direction, the electrical conductivity is as low as less than 35% IACS.

Heretofore, however, press forming such as bending of a Cu-Ni-Sn-P-based alloy sheet which becomes a raw material of the connection component such as automotive terminal or connector is mostly performed under working conditions in a relatively low-speed deformation region where the sheet is less subject to a large strain rate. As a result, even when elongation of the conventional Cu-Ni-Sn-P-based alloy is low as described above, generation of various shaping defects such as cracking can be suppressed by virtue of, for example, mild or devised working conditions and there are not caused many troubles in the working into a terminal or a connector.

Meanwhile, the process of press-forming a copper alloy sheet and producing a connection component such as automotive terminal or connector shown in Fig. 4 recently has also become higher and higher in the efficiency and speed. In such high-efficiency and high-speed press forming, during bending work such as 180° contact bending or 90° bending after notching, the sheet is irresistibly subject to a large strain rate and under working conditions in a high-speed deformation region with such a large strain rate, various shaping defects such as cracking are readily generated. To avoid this problem, high formability, that is, a higher elongation value, is required for the raw material copper alloy sheet.

However, there is a high possibility that conventional Cu-Ni-Sn-P-based alloys with low elongation cannot cope with the high-efficiency high-speed press forming to thereby cause various shaping defects such as cracking. This generation of shaping defects not only reduces the yield of the shaped article but also could be a serious problem in the production line, such that the high-efficiency high-speed press forming process (line) is stopped on every occurrence of a shaping defect.

Conventional Cu-Ni-Sn-P-based alloys have low elongation as described above or techniques for enhancing the elongation characteristic itself are not found, and therefore, the number of cases disclosing the elongation value itself is few. In this respect, the elongation value is exceptionally disclosed in Examples (Tables) of Japanese Patent No. 3,871,064 and JP-A-2002-294368. In Japanese Patent No. 3,871,064, taking a most excellent example with an elongation of 10.1%, the 0.2%-proof stress as the mechanical properties is 521 MPa, the stress relaxation ratio is 12.7% in the direction parallel to the rolling direction, and the electrical conductivity is 31.2% IACS. In JP-A-2002-294368, taking a most excellent example with an elongation of 9.1%, the 0.2%-proof stress as the mechanical properties is 530 MPa, the stress relaxation ratio is 9.8% in the direction parallel to the rolling direction, and the electrical conductivity is 33.2% IACS.

Accordingly, it is corroborated by these Japanese Patent No. 3,871,064 and JP-A-2002-294368 that, as described above, in conventional Cu-Ni-Sn-P-based alloys, when the 0.2%-proof stress is about 500 MPa, the elongation is less than 10% and not high for the strength and also, despite a stress relaxation ratio of 15% or less, the electrical conductivity is not high.

To cope with this, a Cu-Ni-Sn-P-based alloy sheet having a higher elongation value responsive to the above-described high-efficiency high-speed press forming process for producing a connection component such as automotive terminal or connector is demanded. Moreover, this copper alloy sheet needs to satisfy not only elongation but also other properties required for a connection component such as automotive terminal or connector.

That is, there is demanded a Cu-Ni-Sn-P-based alloy sheet having, as terminal/connector properties, an electrical conductivity of 32% IACS or more and a stress relaxation ratio in the direction parallel to the rolling direction of 15% or less and further having, as mechanical properties, a 0.2%-proof stress of 500 MPa or more and an elongation of 10% or more.

In view of these points, a first object of the present invention is to provide a Cu-Ni-Sn-P-based alloy sheet with excellent strength-ductility balance, which is responsive to the above-described high-efficiency high-speed press forming process for producing a connection component such as automotive terminal or connector and also satisfies the properties required for a terminal or connector.

Meanwhile, the stress relaxation ratio of a rolled copper alloy sheet (obtained by rolling) has anisotropy and takes a different value according to the direction in which the longitudinal direction of the female terminal 3 in Fig. 4 runs with respect to the rolling direction of the raw material copper alloy sheet. The same applies to the measurement of the stress relaxation ratio, and the measured stress relaxation ratio takes a different value according to the direction in which the longitudinal direction of a test specimen runs with respect to the rolling direction of the raw material copper alloy sheet. Accordingly, the stress relaxation ratio is liable to be low in the orthogonal direction than in the parallel direction with respect to the rolling direction of the copper alloy sheet.

In this respect, at the time of press working a raw material copper alloy sheet to produce a female terminal 3 in Fig. 4, blanking is sometimes performed such that the longitudinal direction of the female terminal 3 (the longitudinal direction of the pressing strip 5) runs in the direction orthogonal to the rolling direction. A high stress relaxation resistance characteristic is usually required for the bending (elastic deformation) in the length direction of the pressing strip 5. Accordingly, when blanking is performed to allow for running in the direction orthogonal to the rolling direction, it is required to have a high stress relaxation resistance characteristic not in the parallel direction but in the orthogonal direction with respect to the rolling direction of the copper alloy sheet.

In this respect, when the stress relaxation ratio is high in the direction orthogonal to the rolling direction as well as in the direction parallel to the rolling direction, even when the blanking is performed in either one direction of parallel direction and orthogonal direction with respect to the rolling direction, the stress relaxation resistance characteristic as a terminal or connector can be satisfied irrespective of the blanking direction of the raw material copper alloy sheet.

In view of this point, a second object which is not within the scope of the present invention would be to provide a Cu-Ni-Sn-P-based copper alloy sheet with an excellent stress relaxation resistance characteristic, which satisfies, as a terminal or connector, a high stress relaxation ratio in the direction orthogonal to the rolling direction as well as in the direction parallel to the rolling direction.

On the other hand, the conventional Cu-Ni-Sn-P-based copper alloy enhanced in the stress relaxation resistance characteristic is not excellent in bendability or press punchability. The working of a copper alloy sheet into a terminal or connector sometimes involves a severe bending work such as contact bending or 90° bending after notching or a stamping work such as press punching of the sheet, and bendability high enough to withstand such a working or excellent press punchability is becoming required.

However, like conventional Cu-Ni-Sn-P-based alloy enhanced in the stress relaxation resistance characteristic, when the strength is increased, for example, to a 0.2%-proof stress of 500 MPa or more by adding a solid solution strengthening element or increasing the working ratio of cold rolling, deterioration of bendability is inevitably incurred and it is quite difficult to satisfy both of required strength and bendability.

Also, although the usage or alloy system is utterly different, in other copper alloys such as Cu-Fe-P-based copper alloy sheet for use as a lead frame, a technique of controlling the chemical components, for example, adding a small amount of Pb, Ca or the like or dispersing a compound working out to a starting point of fracture, or a technique of controlling a grain size, has been heretofore generally employed as the means for enhancing the press punchability. However, when such a technique is intended to be applied to a Cu-Ni-Sn-P-based copper alloy, there may arise a problem that the control itself is difficult or other properties are deteriorated or that the production cost in turn rises.

In the field of Cu-Fe-P-based copper alloy sheet, many proposals have been made to enhance the press punchability or bendability by taking note of the sheet texture (see, JP-A-2000-328158, JP-A-2002-339028, JP-A-2000-328157 and JP-A-2006-63431). In these techniques, the press punchability is enhanced mainly by controlling the accumulation degree of crystal orientation of the copper alloy sheet.

However, in a Cu-Ni-Sn-P-based copper alloy sheet greatly differing in the alloy system or properties from the Cu-Fe-P system, there have not heretofore been made many proposals on this technique of enhancing the press punchability. The reason therefor is presumed because necessity for or usage requiring enhancement of press punchability of the Cu-Ni-Sn-P-based copper alloy sheet has not conventionally been so pressing.

In view of these points, a third object which is not within the scope of the present invention would be to provide a Cu-Ni-Sn-P-based copper alloy sheet satisfying, as a terminal or connector, the requisite properties such as stress relaxation resistance characteristic and bendability, and a fourth object which is not within the scope of the present invention would be to provide a Cu-Ni-Sn-P-based copper alloy sheet which not only satisfies the properties required for a terminal or connector, such as stress relaxation resistance characteristic, but also is excellent in the press punchability.

In order to achieve the first object of the present invention, the gist of the copper alloy sheet with excellent strength-ductility balance (hereinafter sometimes referred to as a first embodiment of the present invention) is a copper alloy sheet consisting of, in terms of mass%, 0.1 to 3.0% of Ni, 0.01 to 3.0% of Sn and 0.01 to 0.3% of P, and optionally of at least one member selected from the group consisting of, in terms of mass%, 0.5% or less of Fe, 1% or less of Zn, 0.1% or less of Mn, 0.1% or less of Si and 0.3% or less of Mg, optionally of at least one member selected from the group consisting of Ca, Zr, Ag, Cr, Cd, Be, Ti, Co, Au and Pt, in a total amount of 1.0 mass% or less, and optionally of at least one member selected from the group consisting of Hf, Th, Li, Na, K, Sr, Pd, W, S, C, Nb, Al, V, Y, Mo, Pb, In, Ga, Ge, As, Sb, Bi, Te, B and Misch metal, in a total amount of 0.1 mass% or less, with the balance being copper and inevitable impurities, wherein the copper alloy sheet has, as terminal/connector properties, an electrical conductivity of 32% IACS or more and a stress relaxation ratio in the direction parallel to the rolling direction as measured according to SAE standards JASO-C400 after holding at 150°C for 1.000 hr, of 15% or less and further has, as mechanical properties, a 0.2%-proof stress of 500 MPa or more and an elongation of 10% or more, wherein the copper alloy sheet has an intensity peak at the X-ray diffraction angle (2θ) between 100° and 102° in the X-ray diffraction pattern.

As regards preferred properties, the copper alloy sheet has, as terminal/connector properties, an electrical conductivity or 35% IACS or more and a stress relaxation ratio in the direction parallel to the rolling direction of 15% or less and further has, as mechanical properties, a 0.2%-proof stress of 520 MPa or more and an elongation of 12% or more.

The method for producing any one of copper alloy sheets described above or later according to the first embodiment of the present invention comprises casting a copper alloy having any one of compositions described above or later and subjecting the copper alloy ingot to hot rolling, cold rolling and finish annealing in this order to obtain a copper alloy sheet, wherein the finish annealing is performed at a maximum peak temperature of the copper alloy sheet of 500 to 800°C and the average temperature rise rate of the copper alloy sheet to the temperature above is 50°C/s or more, and wherein when cooling the copper alloy sheet to room temperature, the average cooling rate of the copper alloy sheet from 400°C to room temperature is from 40 to 100°C/h, whereby the copper alloy sheet thus obtained has an intensity peak between 100° and 102° of the X-ray diffraction angle (2θ) in the X-ray diffraction pattern, and has, as terminal properties, an electrical conductivity of 32% IACS or more and a stress relaxation ratio in the direction parallel to the rolling direction of 15% or less and further has, as mechanical properties, a 0.2%-proof stress of 500 MPa or more and an elongation of 10% or more.

The present inventors have succeeded in obtaining a copper alloy sheet with excellent strength-ductility balance according to the first embodiment of the present invention by the above-described characteristic control of finish annealing conditions, where the electrical conductivity is enhanced more than the usually expected effect of elevating the electrical conductivity without reducing the strength which usually decreases by the finish annealing and the elongation of the obtained copper alloy sheet is enhanced while maintaining the stress relaxation resistance characteristic. From a commonsense standpoint, the strength after finish annealing usually decreases due to a recovery/recrystallization phenomenon during finish annealing. Nevertheless, under the above-described characteristic control of finish annealing conditions, surprisingly, the strength is not reduced but is maintained and the elongation is rather enhanced. The electrical conductivity is also elevated.

Namely, in the conventional Cu-Ni-Sn-P-based alloy sheet, the elongation is less than 10% despite a 0.2%-proof stress of 500 MPa or more, and the electrical conductivity is less than 35% IACS despite a stress relaxation ratio of 15% or less. On the other hand, according to the first embodiment of the present invention, a novel Cu-Ni-Sn-P-based alloy sheet having, even when the 0.2%-proof stress is 500 MPa or more, an elongation of 10% or more, an electrical conductivity of 32% IACS or more and a stress relaxation ratio of 15% or less is obtained. More excellent properties of this Cu-Ni-Sn-P-based alloy sheet are such that the electrical conductivity is 35% IACS or more, the stress relaxation ratio is 15% or less in the direction parallel to the rolling direction, the 0.2%-proof stress is 520 MPa or more, and the elongation is 12% or more.

This copper alloy sheet with excellent strength-ductility balance according to the first embodiment of the present invention was subjected to systematic analysis and analyzed in detail for the grain shape, analyzable fine crystallized product such as Ni-P compound, the oxide and the like, but to date, a systematic clear distinction in terms of the structure cannot be drawn between the conventional copper alloy sheet and the present invention. The systematic analysis instruments used herein are SEM (scanning electron microscope), TEM (transmission electron microscope) and the like, which are generally used for direct systematic analysis of this type. Of course, the copper alloy sheet compositions investigated are utterly the same Cu-Ni-Sn-P-based alloy and the production conditions are the same conditions except for changing the finish annealing conditions among samples.

Therefore, the present inventors further performed, as the systematic analysis, X-ray diffraction which is special as compared with the direct systematic analysis means, that is, SEM and TEM. As a result, it has been found that, as described later, in the copper alloy sheet with excellent strength-ductility balance according to the first embodiment of the present invention, an intensity peak is present at the X-ray diffraction angle (2θ) between 100° and 102° in the X-ray diffraction pattern, whereas in the conventional Cu-Ni-Sn-P-based alloy sheet, such an intensity peak is not present.

In other words, the present inventors have found that when such an intensity peak is present in a Cu-Ni-Sn-P-based alloy sheet, even with a 0.2%-proof stress of 500 MPa or more, the elongation is 10% or more, the electrical conductivity is 32% IACS or more, and the stress relaxation ratio is 15% or less. The present inventors have also found that when such an intensity peak is not present, like the conventional Cu-Ni-Sn-P-based alloy sheet, the elongation is less than 10% despite a 0.2%-proof stress of 500 MPa or more and the electrical conductivity is less than 32% IACS despite a stress relaxation ratio of 15% or less. That is, in fact, whether or not the alloy sheet is a novel Cu-Ni-Sn-P-based alloy sheet satisfying all of 0.2%-proof stress, elongation, electrical conductivity and stress relaxation resistance characteristic is depending on whether the above-described specific intensity peak is present or not.

The presence of the specific intensity peak, namely, the specific intensity peak at the X-ray diffraction angle (2θ) between 100° and 102°, means that a certain compound is present in the copper alloy sheet texture. The present inventors anticipate that, as described later, this compound is a specific Sn-based compound. However, also as described later, despite various analyses on the relationship between the possible intermetallic compound in this alloy system and the intensity peak position in the X-ray diffraction pattern, what intermetallic compound assumes the above-described specific intensity peak is not clearly known and at present, the anticipation above is only a matter of speculation. Accordingly, how or whether the specific intensity peak contributes to the above-described difference or enhancement in terms of the properties of the Cu-Ni-Sn-P-based alloy sheet is not necessarily clarified.

In this way, although the specific intensity peak above is an important measure of novelty of the copper alloy sheet with excellent strength-ductility balance according to the first embodiment of the present invention, it is not always clear whether the specific intensity peak is an essential requirement to bring out the above-described difference in the properties.

However, according to the first embodiment of the present invention, a Cu-Ni-Sn-P-based alloy sheet with excellent strength-ductility balance, which is responsive to the above-described high-efficiency high-speed press forming process for producing a connection component such as automotive terminal or connector and satisfies also the properties required for a terminal or connector, can be provided.
Fig. 1 shows an explanatory view showing the X-ray diffraction pattern of a copper alloy sheet.
Fig. 2 shows an explanatory view showing the X-ray diffraction pattern of a copper alloy sheet.
Fig. 3 shows cross-sectional views for explaining the stress relaxation resistance test of a copper alloy sheet.
Fig. 4 shows cross-sectional views showing the structure of a box-type connector.
Fig. 5 shows a schematic view showing the half-value breadth of the X-ray diffraction intensity peak.
Fig. 6 shows explanatory views showing the measuring method of a shear plane ratio.

### Description of Reference Numerals and Signs

a: Specific intensity peak between 100° and 102° in the X-ray diffraction pattern
1: test specimen
2: test board
3: box-type connector (female terminal)
4: upper holder part
5: pressing strip
6: male terminal
7: wire connecting part
8: anchoring tongue strip

The present invention is described in detail below. In the context of the present invention, all percentages defined by the mass are the same as those defined by the weight, respectively.

The first embodiment of the present invention is described in detail below.

### (X-Ray Diffraction)

In the first embodiment of the present invention, a specific intensity peak in the X-ray diffraction pattern is specified as an important measure of novelty of a copper alloy sheet with excellent strength-ductility balance. That is, in the X-ray diffraction pattern of the copper alloy sheet, an intensity peak is specified to be present at the X-ray diffraction angle (2θ) between 100° and 102°.

This specific intensity peak is, as described later, presumed to be assignable to an Ni-Sn-based compound, but because of an alloy component or alloy element, the peak height is extremely low as compared with the intensity peak height of Cu which is originally main as the matrix. Whether the degree of this specific peak height contributes to the difference in the properties such as elongation of the Cu-Ni-Sn-P-based alloy sheet is not clearly known as described above. However, also as described above, the properties of the copper alloy sheet can be clearly distinguished from conventional properties of low elongation and low electrical conductivity by whether or not this specific intensity peak is present.

Accordingly, in the first embodiment of the present invention, when it is objectively recognized that an intensity peak rising over fluctuation (variation) of the intensity peak due to noise is substantially present at the X-ray diffraction angle (2θ) between 100° and 102° (in the vicinity of 101°) in the X-ray diffraction pattern, it is specified that the specific intensity peak is present.

### (Figs. 1 and 2)

Fig. 1 shows X-ray diffraction patterns of various copper alloy sheets of Inventive Example 1 and Comparative Examples 20, 22 and 23 in Table 2 in First Example described below, and Fig. 2 shows only the X-ray diffraction pattern of Inventive Example 1 extracted from Fig. 1.

In both of Figs. 1 and 2, the ordinate indicates the X-ray diffraction intensity (CPS) and the abscissa indicates the X-ray diffraction angle (2θ). The X-ray diffraction intensity on the ordinate differs in the range and is from 0 to 1,000 CPS in Fig. 1 and from 0 to 3,500 CPS in Fig. 2. The X-ray diffraction angle also differs in the range and is from 30 to 112° in Fig. 1 and from 80 to 120° in Fig. 2.

In Fig. 1, the top X-ray diffraction pattern is Inventive Example 1, and X-ray diffraction patterns of Comparative Examples 20, 22 and 23 are arranged in this order from the upper side. For the sake of showing these patterns together in the same Fig. 1, each reference line except for Comparative Example 23 is arranged by daringly raising the bank.

In Fig. 1, the X-ray diffraction patterns of various copper alloy sheets of Inventive Example 1 and Comparative Examples have an intensity peak of the main Cu, as shown by the arrow Cu, appearing in the portion of the same X-ray diffraction angle (2θ), because these copper alloys are in the same composition system. The intensity peak position is present between 50° and 51°, between 59° and 60°, between 89° and 90°, and between 110° and 111 °, of the X-ray diffraction angle.

In Fig. 1, the X-ray diffraction pattern of Inventive Example 1 and the X-ray diffraction pattern of each Comparative Example differ only in the point whether or not the specific intensity peak denoted by the arrow a is present at the X-ray diffraction angle (2θ) between 100° and 102°. In Fig. 1 and Fig. 2 extracting only Inventive Example 1, it is objectively recognized only in Inventive Example 1 that an intensity peak rising over fluctuation (variation) due to noise is substantially present.

### (Compound Implied by Intensity Peak)

Usually, a compound (precipitate) having such an intensity peak a (specific peak) appearing at the X-ray diffraction angle (2θ) between 100° and 102° is itself unknown in the Cu-Ni-Sn-P-based alloy. The compound having a closest X-ray diffraction angle is an Ni₃Sn compound (precipitate) oriented in (511) plane. The X-ray diffraction angle of this compound is 102°, and an intensity peak appears at the 102° position. However, this X-ray diffraction angle (2θ) is not between 100° and 102° specified in the first embodiment of the present invention, and the intensity peak position is slightly shifted to the higher angle side.

Incidentally, in Fig. 2, intensity peak positions (X-ray diffraction angles) of other main compounds (precipitates) produced in the Cu-Ni-Sn-P-based alloy are also shown, confirming that the compound (precipitate) of which intensity peak position appears between 100° and 102° is itself unknown. In Fig. 2, the Ni₃Sn compound oriented in (331) plane and the Cu₃Sn compound oriented in (420) plane have an intensity peak position between 81° and 82°. The intensity peak position of the Ni₃Sn compound oriented in (420) plane is in the vicinity of 84°, the intensity peak position of the Cu₃Sn compound oriented in (422) plane is between 91° and 92°, the intensity peak position of the Ni₃Sn compound oriented in (422) plane is in the vicinity of 94°, the intensity peak position of the Cu₃Sn compound oriented in (511) plane is in the vicinity of 99°, the intensity peak position of the Cu₃Sn compound oriented in (440) plane is between 111° and 112°, the intensity peak of the Ni₃Sn compound oriented in (440) plane is between 115° and 116°, and the intensity peak position of the Cu₃Sn compound oriented in (531) plane is in the vicinity of 120°.

Accordingly, the reasonable presumption based on these facts is that the intensity peak position of the compound (precipitate) having the above-described specific intensity peak a, specified in the first embodiment of the present invention, is shifted to the lower angle side and appears between 100° and 102° because a part of Ni in the Ni₃Sn compound (precipitate) is replaced by Cu. That is, the compound (precipitate) of which the X-ray diffraction angle (2θ) appears between 100° and 102° (specific intensity peak a), specified in the first embodiment of the present invention, is considered to be an Sn-based compound containing Ni and Cu resulting from replacement of a part of Ni by Cu (hereinafter sometimes referred to as a specific Sn-based compound). However, as described above, it is not always clear whether the "compound" considered to be this Sn-based compound containing Ni and Cu contributes to the above-described difference in the properties such as elongation of the Cu-Ni-Sn-P-based alloy sheet.

Nevertheless, in fact, the Cu-Ni-Sn-P-based alloy sheet of which intensity peak is present at the X-ray diffraction angle (2θ) between 100° and 102° in the X-ray diffraction pattern of the copper alloy sheet is responsive to the high-efficiency high-speed press forming process for producing a connection component such as automotive terminal or connector, is excellent in the stress relaxation resistance characteristic and electrical conductivity as a terminal or connector, and has excellent strength-ductility balance. Accordingly, in the following, the component composition and production method are described on the presumption that the specific intensity peak a in the X-ray diffraction pattern is assignable to the above-described specific Sn-based compound.

### (Copper Alloy Component Composition)

The component composition of the copper alloy according to the first embodiment of the present invention is described below. In the first embodiment of the present invention, as a premise, the component composition of the copper alloy is, as described above, a Cu-Ni-Sn-P-based alloy allowing for ingot making in a shaft furnace and because of its high productivity, enabling a great cost down.

In order to obtain a copper alloy that is responsive to the high-efficiency high-speed press forming process for producing a connection component such as automotive terminal or connector and satisfies the properties required for a connection component such as automotive terminal or connector and also that is assured of excellent strength-ductility balance and at the same time, excellent in the stress relaxation resistance characteristic and electrical conductivity, the copper alloy fundamentally comprises 0.1 to 3.0% ofNi, 0.01 to 3.0% of Sn and 0.01 to 0.3% of P, with the balance being copper and inevitable impurities. The % indicative of the content of each element means mass%. The alloy elements of the copper alloy are described below by referring to the reasons of addition or restraint.

### (Ni)

Ni is an element necessary for enhancing the strength or stress relaxation resistance characteristic by forming a fine precipitate with P. Also, Ni forms the specific Sn-based compound related to the specific intensity peak in the X-ray diffraction pattern specified in the first embodiment of the present invention. A content of less than 0.1% causes, even by an optimal production method, shortage in the absolute amount of a fine Ni compound of 0.1 µm or less or of Ni contained as a solid solution or in the amount of the specific Sn-based compound. Accordingly, a content of 0.1% or more is necessary for effectively bringing out those effects ofNi.

However, if Ni is excessively contained to exceed 3.0%, a compound such as oxide, crystallized product or precipitate of Ni is coarsened or a coarse Ni compound increases, as a result, the amount of a fine Ni compound or the amount of Ni contained as a solid solution decreases. Also, the coarsened Ni compound becomes a starting point of fracture and leads to reduction not only in the strength or stress relaxation resistance characteristic but also in the elongation. Accordingly, the Ni content is specified to be 0.1 to 3.0%, preferably 0.3 to 2.0%.

### (Sn)

Sn is contained as a solid solution in the copper alloy and thereby enhances the strength. Also, Sn forms the specific Sn-based compound related to the specific intensity peak in the X-ray diffraction pattern, specified in the first embodiment of the present invention. Furthermore, Sn contained as a solid solution in the matrix suppresses the softening due to recrystallization during annealing. If the Sn content is less than 0.01%, the strength-ductility balance cannot be enhanced due to a too small amount of Sn, whereas if the Sn content exceeds 3.0%, not only the electrical conductivity is significantly decreased but also Sn contained as a solid solution is segregated in the grain boundary to reduce the elongation. Accordingly, the Sn content is specified to be 0.01 to 3.0%, preferably 0.1 to 2.0%.

### (P)

P is an element necessary for enhancing the strength or stress relaxation resistance characteristic by forming a fine precipitate with Ni. Also, P acts as a deoxidizing agent. A content of less than 0.01% causes shortage in the P-based fine precipitate particle and therefore, a content of 0.01% or more is necessary. However, if this element is excessively contained to exceed 0.3%, an Ni-P intermetallic compound precipitated particle is coarsened, which leads to reduction not only in the strength or stress relaxation resistance characteristic but also in the hot workability. Accordingly, the P content is specified to be 0.01 to 0.3%, preferably 0.02 to 0.2%.

### (Fe, Zn, Mn, Si and Mg)

Fe, Zn, Mn, Si and Mg are impurities that readily intermix from a molten raw material such as scrap. These elements each produces an effect when contained but generally decreases the electrical conductivity. Also, if the content is increased, ingot making in a shaft furnace becomes difficult. Accordingly, in the case of obtaining a high electrical conductivity, the contents are specified to be 0.5% or less of Fe, 1% or less of Zn, 0.1% or less of Mn, 0.1% or less of Si and 0.3% or less of Mg. In other words, the contents lower than these upper limits are allowable in the first embodiment of the present invention.

Fe elevates the recrystallization temperature of the copper alloy, similarly to Sn. However, if its content exceeds 0.5%, the electrical conductivity decreases. The content is preferably 0.3% or less.

Zn prevents separation of tin plating. However, if its content exceeds 1%, the electrical conductivity decreases and a high electrical conductivity cannot be obtained. Also, in the case of ingot making in a shaft furnace, the content is preferably 0.05% or less. In the temperature region (from about 150 to 180°C) where the alloy sheet is used as an automotive terminal, the effect of preventing separation of tin plating can be obtained even with a content of 0.05% or less.

Mn and Si have an effect as a deoxidizing agent. However, if the content thereof exceeds 0.1%, the electrical conductivity decreases and a high electrical conductivity cannot be obtained. In the case of ingot making in a shaft furnace, the contents are preferably 0.001 % or less of Mn and 0.002% or less of Si.

Mg has an activity of enhancing the stress relaxation resistance characteristic. However, if its content exceeds 0.3%, the electrical conductivity decreases and a high electrical conductivity cannot be obtained. In the case of ingot making in a shaft furnace, the content is preferably 0.001% or less.

### (Ca, Zr, Ag, Cr, Cd, Be, Ti, Co, Au and Pt)

The copper alloy according to the first embodiment of the present invention is allowed to further contain at least one member selected from the group consisting of Ca, Zr, Ag, Cr, Cd, Be, Ti, Co, Au and Pt in an amount of 1.0% or less in terms of a total amount of these elements. These elements have an activity of preventing coarsening of the grain but, if the amount of these elements exceeds 1.0% in total, the electrical conductivity decreases and a high electrical conductivity cannot be obtained. Also, ingot making in a shaft furnace becomes difficult.

In addition, Hf, Th, Li, Na, K, Sr, Pd, W, S, C, Nb, Al, V, Y, Mo, Pb, In, Ga, Ge, As, Sb, Bi, Te, B and Misch metal are also impurities, and the amount of these elements is limited to 0.1% or less in total.

### (Production Method of Copper Alloy Sheet)

The production method of the copper alloy sheet according to the first embodiment of the present invention is described below. In producing the copper alloy sheet according to the first embodiment of the present invention, the production method itself may be an ordinary method except for the conditions in the finish annealing step. That is, a molten copper alloy after adjusting the component composition is subjected to casting, ingot scalping, soaking and hot rolling and then repeatedly to cold rolling and annealing, whereby a final (product) sheet is obtained. However, preferred production conditions for producing the copper alloy sheet according to the first embodiment of the present invention are present, and these are described below.

In casting the above-described copper alloy composition according to the first embodiment of the present invention, high-productivity ingot making in a shaft furnace which is a large-scale melting furnace is possible. However, the time required is preferably as short as possible, such that the time required from the completion of addition of alloy elements to the initiation of casting in the copper alloy melting furnace is within 1,200 seconds and further, the time required from the extraction of ingot out of the ingot heating furnace to the completion of hot rolling is within 1,200 seconds.

By virtue of shortening the time from the completion of addition of alloy elements to the initiation of casting in the copper alloy melting furnace and shortening the time from the extraction of ingot out of the ingot heating furnace to the completion of hot rolling, generation of a coarse Ni compound can be suppressed and at the same time, the amount of a fine Ni compound or the amount of Ni contained as a solid solution can be ensured. In turn, as a premise, the copper alloy sheet can be assured of the electrical conductivity, stress relaxation resistance characteristic and strength.

Incidentally, even when it is intended to control the amount of a fine Ni compound or the amount of Ni contained as a solid solution mainly by the cold rolling conditions or annealing conditions in the later stage, the absolute amount of a fine Ni compound or of Ni contained as a solid solution already becomes small in the previous steps until the completion of hot rolling. Furthermore, in the case where the amount of a coarse Ni compound produced in the previous steps above is large, a fine product precipitated in the cold rolling and annealing steps is trapped by the coarse product and the amount of a fine product independently present in the matrix is more and more reduced. Accordingly, despite the large amount of Ni added, sufficiently high strength and excellent stress relaxation resistance characteristic may not be obtained.

Hot rolling may be performed in an ordinary manner. The inlet-side temperature of hot rolling is approximately from 600 to 1,000°C, and the finishing temperature is approximately from 600 to 850°C. After the hot rolling, water cooling or standing to cool is performed.

Thereafter, cold rolling and annealing are repeatedly performed to obtain a copper alloy sheet having a product sheet thickness. The annealing and cold rolling may be repeated according to the final (product) sheet thickness. In the cold rough rolling, the working ratio is selected so that a working ratio of approximately from 30 to 80% can be obtained in the final finish rolling. In the middle of the cold rough rolling, intermediate recrystallization annealing may be appropriately interposed.

### (Finish Annealing)

In the copper alloy sheet according to the first embodiment of the present invention, as described above, the specific Sn-based compound of which intensity peak position in the X-ray diffraction pattern appears between 100° and 102° is produced by the characteristic control of the finish annealing conditions. As a result, a copper alloy sheet with excellent strength-ductility balance, where the electrical conductivity is enhanced more than the usually expected effect of elevating the electrical conductivity and the elongation of the obtained copper alloy sheet is enhanced while maintaining the stress relaxation resistance characteristic, is obtained without reducing the strength which usually decreases by the finish annealing. From a commonsense standpoint, the strength after finish annealing usually decreases due to a recovery/recrystallization phenomenon during finish annealing. However, under the characteristic control of finish annealing conditions, the strength is not reduced but is maintained and the elongation is rather enhanced. The electrical conductivity is also elevated.

As for the finish annealing temperature, the finish annealing is performed at a maximum peak temperature of 500 to 800°C in terms of the substantial temperature of the sheet, and the holding time in this temperature range is preferably from 10 to 60 seconds. The average temperature rise rate of the sheet to the maximum peak temperature is 50°C/s or more. Additionally, when cooling the sheet to room temperature, the average cooling rate of the sheet from 400°C to room temperature is from 40 to 100°C/h.

If the average temperature rise rate is too low and is less than 50°C/s, an Ni compound (precipitate) such as Ni-P is coarsened during the sheet temperature rise and the sheet cannot satisfy particularly the elongation, strength and stress relaxation resistance characteristic at the same time. The average temperature rise rate is preferably higher, and the upper limit thereof is determined by the equipment capacity of the annealing furnace used for the finish annealing.

Also, if the average cooling rate from 400°C to room temperature is too low and is less than 40°C/h, an Ni compound (precipitate) such as Ni-P is coarsened and the sheet cannot satisfy particularly the elongation, strength and stress relaxation resistance characteristic at the same time. Furthermore, if the average cooling rate is too low, as a serious issue, Ni as a solid solution is consumed preferentially for the growth of a coarsened Ni compound such as Ni-P. Then, the specific Sn-based compound is not produced and the intensity peak is not allowed to be present at the X-ray diffraction angle (2θ) between 100° and 102° in the X-ray diffraction pattern of the copper alloy sheet. The grain is also coarsened and this causes reduction in the strength and elongation.

On the other hand, if the average cooling rate from 400°C to room temperature is too high and exceeds 100°C/h, a fine precipitate may be produced but, as a serious issue, similarly to the case of the average cooling rate being too low, the specific Sn-based compound is not produced and the specific intensity peak in the X-ray diffraction pattern of the copper alloy sheet is not present. In this way, if the average cooling rate from 400°C to room temperature is too low or too high, the elongation and strength in particular are decreased and a copper alloy sheet excellent in the electrical conductivity and strength-ductility balance cannot be obtained, failing in satisfying these properties including the stress relaxation resistance characteristic all at the same time.

At the cooling from the maximum peak temperature, the average cooling rate of the sheet on the high temperature side down to 400°C can be freely selected. However, in view of preventing both reduction in the efficiency of the annealing step and coarsening of the grain size, the average cooling rate is preferably 100°C/h or more.

The strain relief annealing or stabilizing annealing after the final finish cold rolling is preferably performed under the conditions of a substantial temperature of 250 to 450°C x from 20 to 40 seconds. By this annealing, the strain introduced in the final finish rolling can be removed. At the same time, softening of the material does not occur and reduction in the strength can be suppressed.

### Examples

Working examples according to the first embodiment of the present invention are described below. Copper alloy thin sheets were produced using various Cu-Ni-Sn-P-based alloys by varying the composition and finish annealing conditions (continuous annealing) and evaluated for various properties such as electrical conductivity, strength, elongation and stress relaxation resistance characteristic.

More specifically, a copper alloy having a chemical component composition shown in Table 1 was melted in a coreless furnace and then subjected to ingot making by a semicontinuous casting method (cold solidification rate of casting: 2°C/sec) to obtain an ingot of 70 mm (thickness) x 200 mm (width) x 500 mm (length). The obtained ingots were rolled in common under the following conditions to obtain a copper alloy thin sheet. After the surface of each ingot was scalped and heated, the ingot was heated at 960°C in a heating furnace and immediately hot-rolled at a hot rolling finishing temperature of 750°C into a 16 mm-thick sheet, and the sheet was quenched in water from a temperature of 650°C or more.

In this process, the time required from the completion of addition of alloy elements to the initiation of casting in the melting furnace was set to 1,200 seconds or less commonly among respective Examples, and the time required from the extraction out of the heating furnace to the completion of hot rolling was set to 1,200 seconds or less commonly among respective Examples.

After the removal of oxide scales, the sheet was subjected to cold rolling, continuous finish annealing, cold rolling, and strain relief annealing in this order to produce a copper alloy thin sheet. That is, the sheet after primary cold rolling (rough cold rolling, intermediate cold rolling) was scalped. Finish annealing of the sheet was performed in an annealing furnace at the average temperature rise rate, maximum peak temperature and average cooling rate from 400°C to room temperature each shown in Table 2. Incidentally, the cooling from the maximum peak temperature to 400°C was quenching at an average cooling rate of 100°C/s. Also, commonly in respective Examples, the sheet was held at the maximum peak temperature for 20 seconds.

After the finish annealing, finish cold rolling at a rolling reduction of 60% and then, low-temperature strain relief annealing under the conditions of a substantial temperature of 400°C for 20 seconds were performed to obtain a 0.25 mm-thick copper alloy thin sheet.

### (X-Ray Diffraction Pattern)

A test specimen was sampled from each of the thus-obtained copper alloy thin sheets and after the X-ray diffraction pattern of the test specimen surface was measured by an X-ray diffraction analyzer (Model: RINT 1500) manufactured by Rigaku Corporation, the presence or absence of an intensity peak at the X-ray diffraction angle (2θ) between 100° and 102° (in the vicinity of 101°) in the obtained X-ray diffraction pattern was determined. The scan rate was 2°/min and the sampling width was 0.02°.

Incidentally, when it was recognized that an intensity peak rising over fluctuation (variation) of the intensity peak due to noise was substantially present at the X-ray diffraction angle between 100° and 102°, the intensity peak was judged as being present. On the contrary, when it was recognized that only fluctuation (variation) of the intensity peak due to noise was present between those X-ray diffraction angles, the intensity peak was judged as being not present. The results obtained are shown in Table 2.

Also, in each of Examples, a sample was cut out from the obtained copper alloy sheet and subjected to electrical conductivity measurement, tensile test and stress relaxation ratio measurement. The results obtained are also shown in Table 2.

### (Tensile Test)

A test specimen was sampled from the copper alloy thin sheet and machined to produce a JIS No. 5 tensile test specimen such that the longitudinal direction of the test specimen runs in the direction orthogonal to the rolling direction of the sheet material. This test specimen was measured for mechanical properties including elongation under the conditions of room temperature, a test speed of 10.0 mm/min and GL = 50 mm by a universal tester Model 5882 manufactured by Instron Corp. Incidentally, the proof stress is tensile strength corresponding to a permanent elongation of 0.2%.

### (Electrical Conductivity Measurement)

A sample was extracted from the copper alloy thin sheet and measured for the electrical conductivity. In measuring the electrical conductivity of the copper alloy sheet sample, the sheet was worked into a strip-like test specimen of 10 mm (width) x 300 mm (length) by milling and measured for the electrical resistance by a double bridge-type resistance measuring apparatus according to the measuring method of electrical conductivity of nonferrous metal materials specified in JIS-H0505, and the electrical conductivity was calculated according to the average cross-sectional area method.

### (Stress Relaxation Characteristic)

The copper alloy thin sheet was evaluated for the stress relaxation resistance characteristic in the direction parallel to the rolling direction by measuring the stress relaxation ratio in this direction. More specifically, a test specimen was sampled from the copper alloy thin sheet and measured using the cantilever system shown in Fig. 3. A 10 mm-wide strip-like specimen 1 (with the length direction running in the direction parallel to the rolling direction of the sheet material) was cut out and fixed at one end to a rigid test board 2, and deflection in a size of d (= 10 mm) was given to the portion in a span length L of the specimen 1. At this time, L was determined such that a surface stress corresponding to 80% of the proof stress of the material was loaded on the material. After holding in an oven at 180°C for 30 hours, the specimen was taken out, and the permanent distortion δ after removing the deflection d was determined. The stress relaxation ratio (RS) was calculated according to the formula: RS = (δ/d) x 100. Incidentally, holding of 180°C x 30 hours corresponds to holding of almost 150°C x 1,000 hours as calculated using the Larson-Miller parameter.

As apparent from Table 2, in Inventive Examples 1 to 11 using a copper alloy within the composition range of the first embodiment of the present invention in Table 1 (alloy Nos. 1 to 8), the copper alloy sheets are produced within preferred conditions in terms of the average temperature rise rate of finish annealing and the average cooling rate, particularly, from 400°C to room temperature. Also, the heating furnace extraction temperature and the hot rolling finishing temperature are appropriate. Furthermore, the time required from the completion of addition of alloy elements to the initiation of casting in the melting furnace and the time required from the extraction out of the heating furnace to the completion of hot rolling are also short and proper.

Accordingly, in Inventive Examples of Table 2, an intensity peak (the specific intensity peak a in Figs. 1 and 2) is present at the X-ray diffraction angle (2θ) between 100° and 102° in the X-ray diffraction pattern above. Incidentally, Figs. 1 and 2 show the X-ray diffraction pattern of only Inventive Example 1, but in other Inventive Examples, similarly to Inventive Example 1, the specific intensity peak denoted by the arrow a is present at the X-ray diffraction angle (2θ) between 100° and 102°.

In addition, it is presumed that since the copper alloy sheets of Inventive Examples are produced within the above-described preferred conditions, production of a coarse Ni compound such as oxide, crystallized product or precipitate of Ni is suppressed and the amount of a fine Ni compound or the like or the amount ofNi contained as a solid solution can be ensured.

As a result, the copper alloy sheets of Inventive Examples have, as terminal/connector properties, an electrical conductivity of 32% IACS or more and a stress relaxation ratio in the direction parallel to the rolling direction of 15% or less and further has, as mechanical properties, a 0.2%-proof stress of 500 MPa or more and an elongation of 10% or more. That is, the copper alloy sheets of Inventive Examples are assured particularly of high elongation, strength and electrical conductivity and excellent in the balance of electrical conductivity and strength with ductility and also fulfill the standard for the stress relaxation resistance characteristic, revealing that the copper alloy sheet satisfies all of these properties at the same time.

Accordingly, these Inventive Examples have high formability allowing for bending work even in a high-efficiency high-speed press forming process for producing a connection component such as automotive terminal or connector, which requires bending conditions in a high-speed deformation region with a large strain rate.

However, out of Inventive Examples of Table 2, in both of Inventive Example 2 where the average temperature rise rate of finish annealing is the lower limit of 50°C/s and relatively slow, and Inventive Example 3 where the average cooling rate from 400° to room temperature is the lower limit of 40°C/h and relatively slow, the strength, elongation and stress relaxation resistance characteristic all are relatively lower than those in Inventive Examples 1 and 5 where those conditions are appropriate. Also, in Inventive Example 4 where the average cooling rate from 400°C to room temperature is the upper limit of 100°C/h and relatively fast, the elongation in particular is relatively lower than that in Inventive Examples 1 and 5 where the condition above is appropriate.

In Inventive Example 6 of Table 2 (alloy No. 3 of Table 1), the Ni content is the lower limit of 0.1%; in Inventive Example 7 (alloy No. 4 of Table 1), the Ni content is the upper limit of 3.0%; in Inventive Example 8 (alloy No. 5 of Table 1), the Sn content is the lower limit of 0.01%; in Inventive Example 9 (alloy No. 6 of Table 1), the Sn content is the upper limit of 3.0%; in Inventive Example 10 (alloy No. 7 of Table 1), the P content is the lower limit of 0.01%; and in Inventive Example 11 (alloy No. 8 of Table 1), the P content is the upper limit of 0.3%.

Accordingly, in Inventive Examples 6, 8 and 10 of Table 2 where the amount of the main alloy element is the lower limit, particularly, the stress relaxation resistance characteristic and strength are relatively low as compared with Inventive Examples 1 and 5 where the amount of the main alloy element is appropriate. Also, in Inventive Examples 7, 9 and 11 where the amount of the main alloy element is the upper limit, the electrical conductivity, stress relaxation resistance characteristic and elongation are relatively low as compared with Inventive Examples 1 and 5 where the amount of the main alloy element is appropriate.

In Comparative Examples 14 to 19 of Table 2, the production conditions such as finish annealing are within the preferred range and therefore, similarly to Inventive Examples, the intensity peak (the specific intensity peak a in Figs. 1 and 2) at the X-ray diffraction angle (2θ) between 100° and 102° in the X-ray diffraction pattern is present. Nevertheless, due to use of alloy Nos. 11 to 16 of Table 1 which are a copper alloy out of the composition range of the first embodiment of the present invention, any one of the electrical conductivity, stress relaxation resistance characteristic, strength and elongation is significantly inferior to Inventive Examples.

In Comparative Example 14, the Ni content deviates below the lower limit (alloy No. 11 of Table 1) and therefore, the strength, stress relaxation resistance characteristic and elongation are low. In Comparative Example 15, the Ni content deviates above the upper limit (alloy No. 12 of Table 1) and therefore, the strength, stress relaxation resistance characteristic and elongation are low.

In Comparative Example 16, the Sn content deviates below the lower limit (alloy No. 13 of Table 1). Therefore, in Comparative Example 16, the strength, elongation and stress relaxation resistance characteristic are excessively low. In the copper alloy of Comparative Example 17, the Sn content deviates above the upper limit (alloy No. 14 of Table 1) and therefore, the electrical conductivity and elongation are low.

In Comparative Example 18, the P content deviates below the lower limit (alloy No. 15 of Table 1) and therefore, the strength, elongation and stress relaxation resistance characteristic are low. In Comparative Example 19, the P content deviates above the upper limit (alloy No. 16 of Table 1) and therefore, cracking occurred during hot rolling, failing in characterization.

In Comparative Examples 20 to 24 of Table 2, a copper alloy within the composition range of the first embodiment of the present invention in Table 1 is used (alloy Nos. 1 and 2) and other production conditions are within the preferred range, similarly to Inventive Examples. Nevertheless, only the conditions of the finish annealing are out of the preferred range. In Comparative Example 20, the average temperature rise rate of finish annealing is less than the lower limit and is too slow; in Comparative Examples 21 and 22, the average cooling rate from 400°C to room temperature exceeds the upper limit and is too fast; and in Comparative Examples 23 and 24, the average cooling rate from 400°C to room temperature is less than the lower limit and is too slow.

As a result, in Comparative Examples 20 to 24, unlike Inventive Examples, a specific intensity peak a shown in Fig. 1 is not present at the X-ray diffraction angle (2θ) between 100° and 102°. Accordingly, in these Comparative Examples, all of the electrical conductivity, strength and elongation in particular are extremely inferior to Inventive Examples, though the stress relaxation resistance characteristic is rather equal to that in Inventive Examples.

These results reinforce the meanings of the component composition of the copper alloy in the first embodiment of the present invention and the X-ray diffraction pattern, for obtaining a Cu-Ni-Sn-P-based alloy sheet with excellent strength-ductility balance, which is responsive to the high-efficiency high-speed press forming process subject to working conditions in a high-speed deformation region with a large strain rate and satisfies also the properties required for a terminal or connector, and further the meanings of the preferred production conditions for obtaining the X-ray diffraction pattern above.

That is, in the first embodiment of the present invention, a novel Cu-Ni-Sn-P-based alloy sheet having, even when the 0.2%-proof stress is 500 MPa or more, an elongation of 10% or more, an electrical conductivity of 32% IACS or more and a stress relaxation ratio of 15% or less is obtained. As more excellent properties, a Cu-Ni-Sn-P-based alloy sheet having an electrical conductivity of 35% IACS or more, a stress relaxation ratio of 15% or less, a 0.2%-proof stress of 520 MPa or more and an elongation of 12% or more is obtained.

**Table 1**

| Class | No. | Chemical Component Composition of Copper Alloy Sheet (balance: Cu) | | | | | | | | | |
|---|---|---|---|---|---|---|---|---|---|---|---|
| | | Ni | Sn | P | Fe | Zn | Mn | Si | Mg | Element Group A | Element Group B |
| Inventive Example | 1 | 0.8 | 1.1 | 0.07 | 0.02 | 0.04 | - | - | - | - | - |
| | 2 | 1.1 | 0.8 | 0.06 | 0.02 | - | 0.01 | - | 0.01 | - | - |
| | 3 | 0.1 | 1.1 | 0.07 | 0.02 | 0.04 | - | - | - | - | - |
| | 4 | 3.0 | 1.1 | 0.07 | 0.02 | 0.04 | - | - | - | - | - |
| | 5 | 1.1 | 0.01 | 0.06 | 0.02 | - | 0.01 | - | 0.01 | - | - |
| | 6 | 0.5 | 3.0 | 0.04 | 0.02 | - | 0.01 | - | 0.01 | - | - |
| | 7 | 1.1 | 0.8 | 0.01 | 0.02 | - | 0.01 | - | 0.01 | - | - |
| | 8 | 1.1 | 0.8 | 0.3 | 0.02 | - | 0.01 | - | 0.01 | - | - |
| Comparative Example | 11 | 0.04 | 1.1 | 0.07 | 0.02 | 0.04 | - | - | - | - | - |
| | 12 | 3.1 | 1.1 | 0.07 | 0.02 | 0.04 | - | - | - | - | - |
| | 13 | 0.8 | - | 0.07 | 0.02 | 0.04 | - | - | - | - | - |
| | 14 | 0.8 | 3.1 | 0.07 | 0.02 | 0.04 | - | - | - | - | - |
| | 15 | 0.80 | 1.1 | 0.004 | 0.02 | 0.04 | - | - | - | - | - |
| | 16 | 0.80 | 1.1 | 0.35 | 0.02 | 0.04 | - | - | - | - | - |

| | | | | | | | | | | | |
|---|---|---|---|---|---|---|---|---|---|---|---|
| * "-" indicates that the content is below the detection limit. * Other Element Group A: the total content of Ca, Zr, Ag, Cr, Cd, Be, Ti, Co, Au and Pt. * Other Element Group B: the total content of Hf, Th, Li, Na, K, Sr, Pd, W, S, C, Nb, Al, V, Y, Mo, Pb, In, Ga, Ge, As, Sb, Bi, Te, B and Misch metal. | | | | | | | | | | | |

**Table 2**

| Class | No. | Alloy No. of Table 1 | Finish Annealing Conditions | | | X-Ray Diffraction Pattern | Properties of Copper Alloy Sheet | | | | |
|---|---|---|---|---|---|---|---|---|---|---|---|
| | | | Average Temperature Rise Rate (°C/s) | Maximum Peak Temperature (°C) | Average Cooling Rate from 400°C (°C/h) | Presence or Absence of Intensity Peak Near 101° | Electrical Conductivity (%IACS) | Tensile Strength (MPa) | 0.2%-Proof Stress (MPa) | Elongation (%) | Stress Relaxation Ratio (%) |
| Inventive Example | 1 | 1 | 200 | 660 | 70 | present | 40 | 600 | 580 | 13 | 11 |
| | 2 | 1 | 50 | 660 | 70 | present | 41 | 590 | 575 | 12 | 13 |
| | 3 | 1 | 200 | 660 | 40 | present | 42 | 585 | 570 | 12 | 13 |
| | 4 | 1 | 200 | 660 | 100 | present | 39 | 610 | 590 | 11 | 14 |
| | 5 | 2 | 100 | 660 | 50 | present | 43 | 535 | 520 | 14 | 13 |
| | 6 | 3 | 150 | 600 | 70 | present | 40 | 515 | 500 | 15 | 15 |
| | 7 | 4 | 220 | 550 | 70 | present | 35 | 600 | 585 | 12 | 10 |
| | 8 | 5 | 200 | 700 | 70 | present | 45 | 515 | 500 | 14 | 13 |
| | 9 | 6 | 200 | 660 | 70 | present | 30 | 660 | 645 | 10 | 12 |
| | 10 | 7 | 200 | 660 | 70 | present | 44 | 550 | 535 | 13 | 14 |
| | 11 | 8 | 200 | 660 | 70 | present | 35 | 620 | 605 | 12 | 13 |
| Comparative Example | 14 | 11 | 200 | 660 | 70 | present | 38 | 495 | 480 | 9 | 18 |
| | 15 | 12 | 200 | 660 | 70 | present | 32 | 580 | 560 | 7 | 15 |
| | 16 | 13 | 200 | 660 | 70 | present | 47 | 500 | 480 | 8 | 15 |
| | 17 | 14 | 200 | 660 | 70 | present | 28 | 665 | 650 | 7 | 12 |
| | 18 | 15 | 200 | 660 | 70 | present | 45 | 535 | 515 | 9 | 16 |
| | 19 | 16 | 200 | 660 | 70 | present | - | - | - | - | - |
| | 20 | 1 | 30 | 660 | 70 | none | 41 | 580 | 565 | 6 | 13 |
| | 21 | 1 | 200 | 660 | 120 | none | 37 | 570 | 550 | 7 | 12 |
| | 22 | 1 | 200 | 660 | 150 | none | 35 | 550 | 535 | 7 | 11 |
| | 23 | 1 | 200 | 660 | 20 | none | 42 | 530 | 515 | 7 | 13 |
| | 24 | 2 | 200 | 660 | 30 | none | 43 | 520 | 505 | 8 | 14 |

While the present invention has been described in detail and with reference to specific embodiments thereof, it will be apparent to one skilled in the art that various changes and modifications can be made therein without departing from the scope thereof

As described in the foregoing pages, according to the first embodiment of the present invention, a Cu-Ni-Sn-P-based alloy sheet with excellent strength-ductility balance, which is responsive to the high-efficiency high-speed press forming process for producing a connection component such as automotive terminal or connector and satisfies also the properties required for a terminal or connector, can be provided.

Accordingly, the present invention is suitable particularly for a connection component such as automotive terminal or connector.

## Claims

1. A copper alloy sheet consisting of, in terms of mass%, 0.1 to 3.0% of Ni, 0.01 to 3.0% of Sn and 0.01 to 0.3% of P, and optionally of at least one member selected from the group consisting of, in terms of mass%, 0.5% or less of Fe, % or less of Zn, 0.1 % or less of Mn, 0.1 % or less of Si and 0.3% or less of Mg, optionally of at least one member selected from the group consisting of Ca, Zr, Ag, Cr, Cd, Be, Ti, Co, Au and Pt, in a total amount of 1.0 mass% or less, and optionally of at least one member selected from the group consisting of Hf, Th, Li, Na, K, Sr, Pd, W, S, C, Nb, Al, V, Y, Mo, Pb, In, Ga, Ge, As, Sb, Bi, Te, B and Misch metal, in a total amount of 0.1 mass% or less, with the balance being copper and inevitable impurities, wherein the copper alloy sheet has, as terminal/connector properties, an electrical conductivity of 32% IACS or more and a stress relaxation ratio in the direction parallel to the rolling direction, as measured according to SAEJ Standards JASO-C400 after holding at 150°C for 1,000 hr, of 15% or less and further has, as mechanical properties, a 0.2%-proof stress of 500 MPa or more and an elongation of 10% or more, wherein the copper alloy sheet has an intensity peak at the X-ray diffraction angle (2θ) between 100° and 102° in the X-ray diffraction pattern.

2. The copper alloy sheet as claimed in claim 1, wherein the copper alloy sheet has an electrical conductivity of 35% IACS or more and further has, as mechanical properties, a 0.2%-proof stress of 520 MPa or more and an elongation of 12% or more.

## Patentansprüche

1. Kupferlegierungsblech, bestehend aus, in Form von Masse-%, 0,1 bis 3,0% von Ni, 0,01 bis 3,0% von Sn und 0,01 bis 0,3% von P, und gegebenenfalls aus mindestens einem Element, ausgewählt aus der Gruppe, bestehend aus, in Form von Masse-%, 0,5% oder weniger von Fe, 1% oder weniger von Zn, 0,1% oder weniger von Mn, 0,1% oder weniger von Si und 0,3% oder weniger von Mg, gegebenenfalls aus mindestens einem Element, ausgewählt aus der Gruppe, bestehend aus Ca, Zr, Ag, Cr, Cd, Be, Ti, Co, Au und Pt; in einer Gesamtmenge von 1,0 Masse-% oder weniger, und gegebenenfalls aus mindestens einem Element, ausgewählt aus der Gruppe, bestehend aus Hf, Th, Li, Na, K, Sr, Pd, W, S, C, Nb, Al, V, Y, Mo, Pb, In, Ga, Ge, As, Sb, Bi, Te, B und Mischmetall, in einer Gesamtmenge von 0,1 Masse-% oder weniger, wobei der Rest Kupfer und unvermeidbare Verunreinigungen ist, wobei das Kupferlegierungsblech, als Anschluss-/Verbindungsteileigenschften, ein elektrische Leitfähigkeit von 32% IACS oder mehr und ein Spannungsentladungsverhältnis in der Richtung parallel zur Laufrichtung, gemessen gemäß SAEJ Standards JASO-C400 nach dem Halten bei 150°C für 1.000 Stunden, von 15% oder weniger aufweist, und ferner, als mechanische Eigenschaften, eine 0,2%-Dehngrenze von 500 MPa oder mehr und eine Dehnung von 10% oder mehr aufweist, wobei das Kupferlegierungsblech in dem Röntgenbeugungsmuster einen Intensitätspeak bei dem Röntgenbeugungswinkel (2θ) zwischen 100° und 102° aufweist.

2. Kupferlegierungsblech nach Anpruch 1, wobei das Kupferlegierungsblech eine elektrische Leitfähigkeit von 35% IACS oder mehr aufweist und ferner, als mechanische Eigenschaften, eine 0,2%-Dehngrenze von 520 MPa oder mehr und eine Dehnung von 12% oder mehr aufweist.

## Revendications

1. Un feuille en alliage de cuivre consistant en, exprimé en % massique, 0.1 à 3.0% de Ni, 0.01 à 3.0% de Sn et 0.01 à 0.3% de P, et optionnellement au moins un élément sélectionné dans le groupe consistant en, exprimé en % massique, 0.5% ou moins de Fe, % ou moins de Zn, 0.1% ou moins de Mn, 0.1% ou moins de Si et 0.3% ou moins de Mg, optionnellement au moins un élément sélectionné dans le groupe consistant en Ca, Zr, Ag, Cr, Cd, Be, Ti, Co, Au et Pt dans une quantité totale de 1.0% ou moins, et optionnellement au moins un élément sélectionné dans le groupe consistant en Hf, Th, Li, Na, K, Sr, Pd, W, S, C, Nb, Al, V, Y, Mo, Pb, In, Ga, Ge, As, Sb, Bi, Te, B et mischmétal, dans une quantité totale de 0.1% ou moins, le reste étant du cuivre et d'inévitables impuretés, dans lequel la feuille en alliage de cuivre a, comme propriétés de terminal/connecteur, une conductivité électrique de 32% ou plus selon le IACS (International Annealed Copper Standard) et un rapport de relaxation à la contrainte dans une direction parallèle à la direction de laminage de 15% ou moins, tel que mesuré selon les standards JASO-C400 du SAEJ (Society of Automotive Engineers of Japan) après un maintien à 150°C pour 1000 heures et a en outre, comme propriétés mécaniques, une limite d'allongement à 0.2% de 500 MPa ou plus et une élongation de 10% ou plus, dans lequel la feuille en alliage de cuivre a un pic d'intensité à un angle de diffraction (2θ) des rayon X entre 100° et 102° dans le diagramme de diffraction des rayons X.

2. La feuille en alliage de cuivre selon la revendication 1, dans lequel la feuille en alliage de cuivre a une conductivité électrique de 35% ou plus selon le IACS et a en outre, comme propriétés mécaniques, une limite d'allongement à ≥ de 520 MPa ou plus et une élongation de 12% ou plus.
